

# UNITED STATES PATENT OFFICE.

JOHN W. GILBERT, OF WINDSOR, VERMONT, ASSIGNOR OF ONE-HALF TO DANIEL H. PARKER, OF WINDSOR, VERMONT.

## PROCESS FOR HARDENING STEEL.

1,275,242.

Specification of Letters Patent. Patented Aug. 13, 1918.

No Drawing.

Application filed May 8, 1916. Serial No. 96,043.

To all whom it may concern:

Be it known that I, JOHN W. GILBERT, a citizen of the United States, residing at Windsor, in the county of Windsor and 5 State of Vermont, have invented a new and useful Improvement in Processes for Hardening Steel, of which the following is a specification.

My improved process for hardening steel 10 is particularly adapted for hardening and tempering of those steel alloys now in common use, and known as high speed steel, and it consists in certain improvements therein, as are hereinafter described and pointed 15 out in the annexed claims.

It has been found in practice that certain 20 alloys of steel forming that quality now commonly used for cutting tools, and known as high speed steel, require a special treatment to render them sufficiently tough to prevent the cracking of the tool, and at the same time secure a cutting edge of sufficient 25 resistance.

In carrying my improved process into 25 practice, I first heat the steel to be treated to a temperature of about 700° Fahrenheit by subjecting it to a heating medium but little, if any, above the desired heat to which the steel is to be brought, thereby

30 causing the heat diffusion to take place slowly. When the steel has reached a degree of approximately 700° Fahrenheit, I subject it to a heating medium of greater intensity to cause the heating to take place 35 with greater rapidity until the steel reaches a temperature of about 1500° Fahrenheit. The steel is then brought with greater rapidity to a temperature of from 2000° to 2500° Fahrenheit.

40 By the above process, the heating of the steel is accomplished progressively, and I secure this result by placing the steel successively in furnaces of different temperatures, or by moving it in the same furnace from one position to another, successive positions having greater heat intensity.

I next cool the heated steel in a metal bath heated to between 700° and 1500° Fahrenheit. The heated steel is retained in the 50 metal bath until it has reached the temperature of the bath. It is then withdrawn and cooled in the air to a temperature less than 200° Fahrenheit. The temper is then drawn in a bath preferably 55 of melted tallow of a temperature ranging

from 500° upward Fahrenheit, this temperature depending upon the purpose for which the steel is to be used, and the size of the article tempered.

I am aware that in some processes of 60 tempering steel, metal baths, such as aluminum, lead, or tin baths, have been used, and I do not therefore claim broadly the use of a metal bath.

In carrying my process into practice I 65 prefer to use a metal bath of melted lead heated above the temperature of the melting point, and the steel is immersed in this bath until it acquires substantially the temperature of the bath, which sufficiently 70 hardens the steel without cracking it.

I am aware that steel has been treated by heating it to a cherry red and immersing it in a bath of melted lead or tin. By my process the immersion in the lead bath 75 becomes a cooling process owing to the high temperature at which the steel is preheated, and the lead bath is superior to other cooling baths now in use owing to its greater conductivity. I am also aware that it has 80 been a common practice to harden steel by heating and rapidly cooling it, and to finally draw the temper by immersing the steel in a bath of oil.

In the use of what are known as high 85 speed steels containing tungsten or other alloy, there is great liability of cracking, and it is difficult to obtain the necessary hardness combined with the required toughness which is secured by my process.

The variations in temperature noted in the several steps of my process are determined by the quality of the steel and the character of the article to be treated, and the use for which it is designed.

I claim,

1. The process of treating high speed steel, comprising slowly heating the steel to a temperature of about 700° Fahrenheit, then heating the steel at a more rapid rate 100 to approximately 1500° Fahrenheit, then heating the steel at a still more rapid rate to a maximum of 2000° to 2500° Fahrenheit, cooling in a metal bath to between 700° and 1500° Fahrenheit and finally cooling in air to 200° or less Fahrenheit.

2. The process of treating high speed steel, comprising progressively heating at different rates of heating, as follows, slowly heating to about 700° Fahrenheit, increas-

ing the rate of heating to about 1500° Fahrenheit, next increasing the rate of heating to about 2000° to 2500° Fahrenheit, cooling in a metal bath to between 700° and 1500° Fahrenheit, and air cooling to approximately room temperature.

3. The within described method of treating high speed steel, comprising progressively heating the steel to a maximum temperature of 2000° to 2500° Fahrenheit, im-

mersing in a metal bath heated to 700° to 1500° Fahrenheit until the steel reaches the temperature of the bath, air cooling the steel and drawing it to the temper desired in an oleaginous bath.

15

Dated this third day of May 1916.

JOHN W. GILBERT.

Witnesses:

H. A. WILLIAMS,  
GLENN C. HOWLAND.